

Nov. 25, 1941

R. S. DEAN

2,263,571

ELECTRICAL RESISTANCE ELEMENT

Filed April 13, 1939

Fig. 1.



Fig. 2.



Inventor:

Reginald S. Dean

By McLaughlin Wallenstein

Atlys

## UNITED STATES PATENT OFFICE

2,263,571

## ELECTRICAL RESISTANCE ELEMENT

Reginald S. Dean, Washington, D. C., assignor to  
Chicago Development Company, Chicago, Ill.,  
a corporation of Illinois

Application April 13, 1939, Serial No. 267,707

7 Claims. (CL 201—76)

This invention relates to electrical resistance elements prepared from alloys of manganese and copper which may be worked into suitable shapes, such as wire, for use in electrical circuits where various combinations are desired of electrical resistance and temperature coefficients of this electrical resistance, with mechanical properties such as high strength and modulus of elasticity.

In my copending application, Serial No. 230,209, filed September 16, 1938, I have disclosed that certain copper-manganese alloys possess great electrical resistance and low temperature coefficients. The present invention relates to methods of obtaining any desired combination of various mechanical and electrical properties by a selection of composition, heat and mechanical treatment of manganese-copper alloys. As set forth in my copending application, the electrical properties of copper-manganese alloys made from electrolytic manganese or substantially pure manganese differ greatly from those of the prior art which are made from commercial manganese containing silicon, aluminum and the like. I have found that, by the use of electrolytic manganese or other manganese of like purity, alloys are produced which are ductile throughout the entire range from 98% to 0% manganese. The alloys containing less than 10% of copper are much more ductile when quenched from a temperature of 1000 degrees C.

In Fig. 1, I have plotted the electrical resistances and temperature coefficients of copper-manganese alloys in various states of mechanical and heat treatment. It will be seen from this diagram that, by the practice of my invention, I produce quenched and cold-worked alloys of approximately equal parts of copper and manganese having specific resistances of more than  $200 \times 10^{-6}$  ohms/cm.<sup>2</sup>. For purposes of comparison, it may be pointed out that the highest resistances which have been heretofore recorded in the work of other investigators which has come to our attention is  $134 \times 10^{-6}$  ohms/cm.<sup>2</sup>. This increase in resistance, which is of great importance in electrical circuits, is obtained by the use of high purity manganese and by the quenching treatment which I have described. The temperature coefficient of electrical resistance of the alloys made in accordance with my invention and quenched or quenched and cold worked is very low throughout the composition range from 20 to 70% manganese. The advantages of being able to combine very high specific resistance with a very low temperature coefficient as is possible by the application of my invention will be evident

to those accustomed to working with electrical circuits.

For certain purposes, it is desirable to obtain increased hardness in electrical resistance alloys. This may be accomplished by cold work by which means the hardness of alloys throughout the range may be considerably increased without greatly affecting their electrical resistance or temperature coefficient. However, when it is desirable to obtain a maximum of hardness, I subject the alloys of my invention to heat treatment at approximately 500 degrees C. for one-half hour after quenching from 1000 degrees and cold working.

In Fig. 2 I have plotted the hardness of the copper-manganese alloys which can be obtained by the various treatments which I have described. It will be seen that with high manganese alloys, it is possible to obtain hardness of more than 20 Rockwell C-40 combined with an electrical resistance of greater than  $100 \times 10^{-6}$  ohms/cm.<sup>2</sup>.

What I claim as new and desire to protect by Letters Patent of the United States is:

1. An electrical resistance element, having a specific resistance of at least about  $150 \times 10^{-6}$  ohms per cm.<sup>2</sup>, said element being made from an alloy selected from the group consisting of quenched and quenched and cold worked alloys consisting substantially entirely of manganese and copper, said alloys containing from about 22% to about 85% manganese.

2. An electrical resistance element having a hardness of at least Rockwell C-20 and an electrical resistance of at least  $100 \times 10^{-6}$  ohms/cm.<sup>2</sup>, said element being made from an alloy consisting substantially entirely of manganese and copper, said alloy containing from about 80% to about 97% manganese.

3. An electrical resistance element in accordance with claim 1 wherein the manganese is electrolytic manganese.

4. An electrical resistance element in accordance with claim 2 wherein the manganese is electrolytic manganese.

5. An electrical resistance element made from an alloy selected from the group consisting of quenched and quenched and cold worked copper-manganese alloys having a specific resistance in excess of  $150 \times 10^{-6}$  ohms per cm.<sup>2</sup>, the manganese being present in proportions ranging from about 26% to about 75%, the balance being substantially copper.

6. A resistance element comprising a copper-manganese alloy having between about 20% and 85% manganese, balance substantially copper,

quenched from a high temperature but below the melting point of the alloy, and having a specific electrical resistance not substantially less than about  $150 \times 10^{-6}$  ohms/cm.<sup>3</sup>

7. An electrical resistance element, said element being made from an alloy quenched from a relatively high temperature but below its melt-

ing point and consisting substantially entirely of copper and manganese, said alloy having a specific resistance of at least  $150 \times 10^{-6}$  ohms per cm.<sup>3</sup>, said alloy containing between 40% and 50% manganese, balance copper.

REGINALD S. DEAN.